

Aug. 28, 1951

R. CAMPBELL ET AL  
METHOD OF INSOLUBILIZING ARTIFICIAL FILAMENTS  
OF VEGETABLE PROTEIN  
Filed July 28, 1948

2,565,908



## UNITED STATES PATENT OFFICE

2,565,908

## METHOD OF INSOLUBILIZING ARTIFICIAL FILAMENTS OF VEGETABLE PROTEIN

Ray Campbell, Ardrossan, William E. Tetlow, Saltcoats, and Robin H. K. Thomson, Fairlie, Scotland, assignors to Imperial Chemical Industries Limited, a corporation of Great Britain

Application July 28, 1948, Serial No. 41,126  
In Great Britain October 6, 1947

6 Claims. (Cl. 8—127.6)

1

The present invention relates to a new or improved method for insolubilising artificial filaments, threads, fibres and the like filamentary products spun from protein solutions, and more particularly those obtained by the spinning of solutions of vegetable seed globulins, for instance peanut protein, or phospho-proteins, for instance casein, in aqueous alkaline or other suitable aqueous solvent media into suitable acidified saline coagulating baths. Sodium sulphate solutions slightly acidified with sulphuric acid are in practice most advantageously used as the coagulating baths.

The filamentary products emerging from the coagulating bath are still easily soluble in dilute saline solutions. They can be rendered insoluble in dilute saline solutions and in cold water by a "hardening" treatment with formaldehyde, but in order to render the filamentary products capable of ordinary textile application they must be rendered capable of withstanding also the action of boiling water, so that they can be dried off without sticking together, and further the action of hot dilute acid solutions such as are used in the application of acid wool dyes and of hot dilute alkaline solutions such as are used in laundering.

While a number of processes for insolubilising protein artificial filamentary products for this purpose have been described it is believed that the best insolubilisation and the best physical properties and separation of the individual filaments or the like from one another have hitherto been attained by the use of a strongly saline solution of formaldehyde containing not less than 30 parts sodium chloride per 100 parts water by weight, acidified with sufficient hydrochloric acid or sulphuric acid to bring the pH below 1. Such a bath is described in British Specification No. 513,910. The coagulating solution associated with the filaments or the like emerging from the coagulating bath is usually rinsed away from them by treating them with sodium chloride brine before introducing them into the aforementioned insolubilising solution.

The insolubilisation with the aforesaid acidified brine formaldehyde solution however necessitates the maintenance of the filamentary product in contact with the insolubilising solution for a prolonged period, even at raised temperatures, for instance 18 hours at 38° C., and the period of treatment cannot be reduced by the employment of considerably higher temperatures, since the loose filaments, threads, fibres tend to clump together at such higher temperatures instead of remaining open.

2

In British Patent Specification No. 597,497, which corresponds to the co-pending U. S. application, Ser. No. 681,153, now U. S. Patent No. 2,533,297, there is claimed a method of insolubilising artificial filamentary products obtained by the spinning of solutions of vegetable seed globulins, for instance, peanut proteins, or phospho-proteins, for instance casein, in aqueous alkaline or other suitable aqueous solvent media into suitable acidified saline coagulating baths by treating the said filamentary products in an aqueous formaldehyde bath saturated to both sodium chloride and sodium sulphate or to both sodium chloride and magnesium sulphate, at a pH of 4 to 6 and at a temperature not exceeding 60° C. and thereafter treating the filamentary product in an aqueous formaldehyde bath strongly acidified with sulphuric acid, that is, containing at least 175 grams of sulphuric acid per litre of solution, and saturated with sodium sulphate or magnesium sulphate at the temperature employed, the said strongly acidified formaldehyde bath being at a raised temperature.

It is stated therein that if the formaldehyde bath of pH 4 to 6 is saturated to both sodium chloride and sodium sulphate then the strongly acidified formaldehyde bath is preferably saturated with sodium sulphate, while if the formaldehyde bath of pH 4 to 6 is saturated to both sodium chloride and magnesium sulphate then the strongly acidified formaldehyde bath is preferably saturated with magnesium sulphate.

It is also stated therein that if the temperature of the first bath is 50° C. a period of about five minutes is sufficient and that if the temperature is about 40° C. 8 minutes to 15 minutes are required. It is also stated that if the temperature of the second bath is about 70° C. the time required for treatment is usually about 10 to 15 minutes.

The object of the present invention is to provide a simple and efficient method of insolubilising a continuous travelling tow of unhardened protein artificial filamentary material.

It has now been found that if the formaldehyde solution at pH 4 to 6 saturated with sodium chloride is at a temperature between 60-70° C. and the treatment is carried out while the tow is passed through a current of the solution in a length of tubing of suitable diameter preferably arranged as a coil of helical form that the solution need not be saturated with respect to sodium sulphate and that the time required for treatment is only about  $\frac{1}{2}$  to 1 minute. It has also been found that if the aqueous formaldehyde solution strongly acidified with sulphuric

acid, that is, containing at least 175 grams of sulphuric acid per litre of solution, and saturated with sodium sulphate or magnesium sulphate at the temperature employed as used in the method of British Patent No. 597,497 is at a temperature of about 95° C. and the treatment is likewise carried out in a current of this solution while passing through a helical tube that the time of treatment required is only about 2 minutes.

According to the present invention the method of insolubilising artificial filamentary products obtained by the spinning of solution of vegetable seed globulins, for instance, peanut proteins, or phospho-protein, for instance, casein in aqueous alkaline or other aqueous solvent media into acidified saline coagulating baths comprises passing the filamentary products and an aqueous formaldehyde solution saturated to sodium chloride and containing sodium sulphate or magnesium sulphate at a pH of 4 to 6 and at a temperature preferably in the neighbourhood of about 70° C. through a tubular passage preferably arranged as a coil of helical form and thereafter passing the thus treated filamentary product and an aqueous formaldehyde solution strongly acidified with sulphuric acid and saturated with sodium sulphate or magnesium sulphate at the temperature employed, the said strongly acidified formaldehyde solution being at raised temperature preferably in the neighbourhood of about 95° C., through another tubular passage preferably arranged as a coil of helical form.

The tubular passage is preferably likewise of narrow diameter and if it is straight the treating liquid is passed therethrough preferably under such conditions as to be in turbulent flow. The treating liquid is always to flow through the tubular passage at least at such speed as to advance the filamentary products through the said passage.

The tubular passage can be completely immersed in a bath of water of such temperature as to maintain the liquor circulating in the passage at the stated temperature and so prevent cooling and consequent crystallisation of salts which might result in damage to the fibre.

The tow of filaments is preferably carried into the tubular passage by having a funnel fitted on to the entrance to the passage. The treating liquor is directed into this funnel, flowing by gravity through the said tubular passage. The flow of liquor from the funnel to the tubular passage provides the necessary impetus to take the tow of filaments into the tubular passage. It has been found advantageous to fit an overflow pipe from the funnel to the treating liquor circulating tank in order to maintain steady flow conditions in the tubular passage.

The invention is further illustrated by the following example in which the parts are parts by weight except where otherwise indicated and with reference to the accompanying diagrammatic drawing.

#### Example

A matured caustic soda solution of groundnut globulin prepared from a solution containing 25 parts peanut globulin, 1.25 parts sodium hydroxide, 1.0 part sodium sulphite and 72.75 parts water is extruded through a spinneret 1 into a coagulating bath 2 containing 200 gm./l. sodium sulphate and 20 gm./l. sulphuric acid. The resulting tow of filaments 3 is taken up on godets 4 having a peripheral speed of 30 metres per minute and stretched by passing on to godets 5

having a peripheral speed of 45 metres per minute.

The tow 3 is then led under tension to a godet 6 situated vertically above the centre line of the trough of a ring-trough 7 in accordance with the method claimed in co-pending U. S. application Serial No. 2,246, filed January 14, 1948, now Patent No. 2,555,065, through a reciprocating spacing device 8 at least 3 feet above the surface 10 of the liquor in the trough and so into the trough in which the fibre is deposited in a zig-zag manner. This ring-trough consists of a solid centre section 2 feet in diameter with a trough 0.5 foot wide and 4 inches deep outside but integrally 15 joined to it and is made of mild steel. The ring trough contains a base of wire gauze 9 and revolves in a circular trough 10, 3 feet 4½ inches external diameter, 1 foot 7½ inches internal diameter and 6" deep, also of mild steel, fitted 20 with an adjustable weir so that the height of liquor in the trough may be varied at will. The ring-trough contains a saturated solution of sodium chloride at a temperature of 20° C. and is at a pH of 5.0. The tow 3 sinks on to the base 9 25 of the trough 7 and is carried round with the trough 7 which revolves one in 4½ minutes. Thus the time of immersion of the tow 3 in the acidified saturated sodium chloride solution is 4½ minutes. The tow 3 is taken up not less than 30 3" from the fibre inlet and then stretched between two godets 11 and 12 whose peripheral speeds are 35 and 52 metres per minute respectively.

After stretching, the tow 3 passes over a godet 35 13 placed vertically above the centre line of the entry 14 of a vertically positioned helical coil 15 of 60-120 feet in length and of 4 feet diameter. Through this coil there passes a solution saturated with respect to sodium chloride at 70° C. and containing 20 grams of sodium sulphate per litre and 2% of formaldehyde. The temperature 40 of this solution is 70° C. and the pH 5.0. The time of passage of the tow 3 through this coil is ½ to 1 minute. The tow 3 is picked up over a godet 16 arranged vertically above the exit of the vertically positioned coil. The tow 3 is stretched 45 between two godets 17, 18 whose peripheral speeds are 40 and 45 metres/minute. The tow 3 then enters through entry 19 another vertically positioned coil 20 of length 150 feet and of diameter 50 4 feet through which flows a treating liquor consisting of saturated sodium sulphate at 95° C., 275 grams per litre sulphuric acid and 2% formaldehyde. The temperature of this liquor is 95° 55 and the pH is less than 0. The time of passage of the tow through this coil 20 is 1-2 minutes. On leaving the outlet of this second coil 20 the tow 3 is taken up over a godet 21 and washed and dried by any known method.

#### We claim:

1. A method for reducing the time of treatment required for insolubilizing artificial filamentary products obtained by spinning aqueous solutions of proteins selected from the group consisting of vegetable seed globulins and phospho-proteins into acidified saline coagulating baths which comprises passing the coagulated filamentary products through a confined area and in direct contact with a stream of an aqueous formaldehyde solution having a temperature of 65 from about 60° C. to 70° C. and a pH of 4 to 6, said solution being saturated with sodium chloride and containing a sulphate from the group 70 consisting of sodium sulphate and magnesium sulphate, and thereafter passing the thus treated 75

filamentary products through another confined area and in direct contact with a stream of a second aqueous formaldehyde solution having a temperature of about 95° C., said last named aqueous formaldehyde solution containing at least 175 grams per litre of sulphuric acid and being saturated, at the temperature employed, with a sulphate from the group consisting of sodium sulphate and magnesium sulphate.

2. The method of claim 1 wherein at least one 10 of said confined areas is of helical form.

3. The method of claim 1 wherein the streams of the aqueous formaldehyde solutions flow in a turbulent manner.

4. The method of claim 1 wherein said filamentary products are in the form of a continuous tow.

5. The method of claim 1 wherein said protein is peanut protein.

6. A method for reducing the time of treatment required for insolubilizing a continuous tow of artificial filamentary products obtained by spinning aqueous solutions of proteins selected from the group consisting of vegetable seed globulins and phospho-proteins into acidified saline coagulating baths which comprises passing said tow in an untensioned condition through a confined area for from about  $\frac{1}{2}$  to 1 minute and in direct contact with a stream of an aqueous formaldehyde solution at a temperature of from about 60° C. to 70° C. having a pH of 4 to 6, said solution being saturated with sodium chloride

and containing a sulphate from the group consisting of sodium sulphate and magnesium sulphate, and thereafter passing the thus treated tow in an untensioned condition through another 5 confined area for about two minutes and in direct contact with a stream of a second aqueous formaldehyde solution at a temperature of about 95° C., said last-named aqueous formaldehyde solution containing at least 175 grams per litre of sulphuric acid and being saturated, at the temperature employed, with a sulphate from the group consisting of sodium sulphate and magnesium sulphate.

RAY CAMPBELL.  
WILLIAM E. TETLOW.  
ROBIN H. K. THOMSON.

#### REFERENCES CITED

20 The following references are of record in the file of this patent:

#### UNITED STATES PATENTS

| Number    | Name         | Date          |
|-----------|--------------|---------------|
| 2,372,622 | Wormell      | Mar. 27, 1945 |
| 2,409,475 | Cline        | Oct. 15, 1946 |
| 2,428,603 | Atwood       | Oct. 7, 1947  |
| 2,429,214 | Biehn et al. | Oct. 21, 1947 |

#### FOREIGN PATENTS

| 30 Number | Country       | Date         |
|-----------|---------------|--------------|
| 543,586   | Great Britain | Mar. 4, 1942 |